

May 21, 1968

D. W. HESELTINE ET AL

3,384,487

BUTADIENYL DYES FOR PHOTOGRAPHY

Filed Sept. 1, 1964

**Fig. 1**



**Fig. 2**



**Fig. 3**



**Fig. 4**



*Donald W. Heseltine  
Jean E. Jones  
Lewis L. Lincoln*  
INVENTORS

BY *R. Frank Smith*  
*Ray Carter Livermore*  
ATTORNEY & AGENT

1

3,384,487

**BUTADIENYL DYES FOR PHOTOGRAPHY**  
Donald W. Heseltine, Jean E. Jones, and Lewis L. Lincoln, Rochester, N.Y., assignors to Eastman Kodak Company, Rochester, N.Y., a corporation of New Jersey  
Filed Sept. 1, 1964, Ser. No. 393,684  
10 Claims. (Cl. 96—84)

## ABSTRACT OF THE DISCLOSURE

Novel indolebutadienyl dyes prepared by reacting an indolinium compound with a cinnamaldehyde compound have valuable light-absorbing characteristics which make them useful in light-sensitive photographic elements and are bleachable. Anhydro-2-(4-p-dimethylaminophenyl-1,1-dimethyl-1,3-butadienyl)-3-(4-sulfobutyl)-1H-benz[e]indolinium hydroxide and 3-carboxyethyl-2-(4-p-dimethylaminophenyl-1,3-butadienyl)-1,1-dimethyl-1H-benz[e]indolinium iodide, for example, are illustrative of the indolebutadienyl dyes.

This invention relates to photography and more particularly to butadienyl dyes and photographic elements containing them.

It is known that light-screening substances are often employed in photographic elements, for example (a) in overcoatings to protect the light-sensitive emulsion from ultraviolet light, especially with color materials, (b) in layers between differentially sensitized emulsions, e.g., to protect red- and green-sensitized emulsions from the action of blue light, and (c) in antihalation layers, on either side of a transparent support carrying the light-sensitive emulsion.

In most cases, and especially when the element contains a color-sensitized emulsion, it is desirable to employ light-screening substances which do not react chemically to affect the general sensitivity or the color sensitivity of light-sensitive emulsions with which they come into contact. It is also desirable to employ light-screening substances which do not diffuse substantially from the layers in which they are incorporated, either during manufacture of the element or during storage. Finally, it is generally necessary to employ light-screening substances which can be decolorized and/or readily removed prior to or during photographic processing; for many purposes it is particularly convenient to employ light-screening substances which are rendered ineffective in one of the photographic processing baths. For example, in an element to be processed by chemical reversal, it may be convenient to employ a light-screening substance which is rendered ineffective (bleached and/or removed) in negative development in order to facilitate exposure of the residual silver halide.

Numerous substances, including many well known dyes, have been employed for light-screening in the applications indicated above, but it has proved extremely difficult to find dyes having the combination of qualities desired. Many are not resistant to diffusion and wander from the layer in which they are coated; many adversely affect the sensitivity of light-sensitive emulsions with which they come into contact. Some are not sufficiently water soluble to enable incorporation into filter layers from aqueous solutions. Some are not bleached or destroyed readily by photographic processing and thus present stain problems in the processed photographic element.

The use of styryl dyes for antihalation protection in backing layers has been known for some time. For example, styryl dyes are disclosed for this purpose in U.S. Patent 1,845,404, issued Feb. 16, 1932. However, few

2

styryl dyes have been found that absorb in the red spectral region, since the high deviations encountered in the dyes from highly basic nuclei reduce markedly the deepening of the color (that is, shift of spectral absorption to longer wave lengths) usually produced by increasing the chain length. Styryl dyes of the indole series are very unstable under even mildly alkaline conditions. Styryl dyes have been prepared previously as light-screening dyes that are soluble in organic solvents, do not wander and are bleachable in conventional processing baths. Many of the prior art dyes have a tendency to precipitate in aqueous solutions of hydrophilic colloids such as gelatin, polyvinyl alcohol, albumen, casein, etc. and the organic solvent, such as, acetone or alcohol allows the dyes to penetrate the support and render the dyes themselves very difficult to bleach or destroy in conventional processing baths.

It is therefore an object of this invention to provide a novel class of butadienyl dyes which are useful in light-sensitive photographic elements.

Another object is to provide for use in filter layers and antihalation layers in photographic elements, a novel class of butadienyl dyes, which not only have valuable light-absorbing characteristics but are more water soluble in neutral or in slightly acid solution than prior art butadienyl dyes and thus are more easily incorporated in the filter layer.

Another object is to provide a novel class of butadienyl light-screening dyes which are less subject to diffusion from the filter layer than are the prior art dyes.

Another object is to provide a novel class of dyes which are bleachable by the photographic developer or fixing solutions during the processing of the photographic element.

Another object is to provide a photographic element having at least one light-sensitive silver halide emulsion layer and at least one light-absorbing filter layer containing a dye selected from the novel class of dyes of our invention.

Still other objects will become apparent from the following description of our invention in the specification and claims.

We have discovered that these and other objects are accomplished by the use of the novel dyes of our invention, which are included in the following formula:

45 I.



wherein L represents the hydrogen atom, or a halogen atom, e.g., chlorine, bromine, fluorine, etc.; Y and Y<sub>2</sub> each represent a member selected from the class consisting of the hydrogen atom and the nonmetallic atoms which together form a fused ring attached to the indolenine ring in the 4 and 5 positions, the 5 and 6 positions, or the 6 and 7 positions; R and R<sub>1</sub> each represent a member selected from the class consisting of the hydrogen atom, an alkyl group, e.g., methyl, ethyl, propyl, butyl, etc., and together represent the nonmetallic atoms necessary to complete a cycloalkane group, e.g., cyclopentane, cyclohexane, etc.; R<sub>2</sub> represents an alkyl group such as, a carboxyalkyl group (e.g. carboxymethyl,  $\beta$ -carboxyethyl,  $\gamma$ -carboxypropyl,  $\delta$ -carboxypentyl,  $\omega$ -carboxypentyl,  $\omega$ -carboxyhexyl, etc.), a hydroxyalkyl group, (e.g.,  $\beta$ -hydroxyethyl,  $\delta$ -hydroxybutyl,  $\omega$ -hydroxyhexyl, etc.), a carboxyalkylcarbamoyloxyalkyl group (e.g., carboxymethylcarbamoyloxyethyl,  $\beta$ -carboxyethylcarbamoyloxyethyl,  $\gamma$ -carboxypropylcarbamoyloxyethyl,  $\omega$ -carboxypentylcarbamoyloxyethyl,  $\beta$ -carboxethyl-

carbamoyloxypropyl, etc.), an alkoxy carbonylalkyl-carbamoyloxyalkyl group (e.g., ethoxycarbonylmethylcarbamoyloxyethyl, methoxycarbonylethylcarbamoyloxyethyl, ethoxycarbonylethylcarbamoyloxyethyl, etc.); a sulfoalkyl group (e.g.,  $\beta$ -sulfoethyl,  $\gamma$ -sulfopropyl,  $\delta$ -sulfovutyl,  $\omega$ -sulfohexyl, etc.); and methyl, ethyl, propyl, butyl, hexyl, etc.;  $X^\ominus$  represents an acid anion, e.g., chloride, bromide, iodide, perchlorate, thiocyanate, benzenesulfonate, methylsulfate, ethylsulfate, p-toluenesulfonate, etc.;  $n$  represents an integer of from 1 to 2 such that  $n$  is 1 only when  $R_2$  contains a carboxy group, and a sulfo group; and  $Z$  represents an aryl group (e.g., a phenyl, a tolyl, a propylphenyl, etc.) substituted with an amino group, such as, the amino group, a dialkylamino group, (e.g., N,N-dimethylamino, N,N-diethylamino, N,N-dipropylamino, N,N-dibutylamino, etc.), an alkylamino group (e.g., N-methylamino, N-propylamino, N-butylamino, etc.), a N-alkyl-N-arylamino group (e.g., N-methyl-N-phenylamino, N-butyl-N-phenylamino, N-ethyl-N-phenylamino, etc.), an alkoxy group (e.g., methoxy, ethoxy, propoxy, butoxy, etc.) and the hydroxy group.

Our dyes are produced to advantage by heating, preferably under reflux, a compound having the formula:

II



with a compound having the formula:

III



dissolved in acetic anhydride. The groups, L, Y, Y2, R, R1, R2, X $\ominus$ , n and Z are as defined previously.

The butadienyl dyes of our invention absorb light of unexpectedly long wavelengths compared either with the corresponding styryl dyes or compared with other butadienyl dyes. Furthermore, our dyes are unexpectedly bleachable in ethylhydroquinone developer solutions compared to butadienyl dyes outside our invention. These properties make our dyes particularly valuable in red-light absorbing backing layers for photographic elements. The acid substituted dyes of our invention are particularly useful with basic vehicles, such as, the cellulose esters of dimethylamino acetic acid.

Among the dyes of our invention are the following typical examples which are intended to illustrate but not limit the scope of our invention.

Dye 1.—Anhydro-2-(4-p-dimethylaminophenyl-1,1-dimethyl-1,3-butadienyl)-3-(4-sulfovutyl)-1H-benz[e]indolium hydroxide



Anhydro-3-(4-sulfovutyl)-1,1,2-trimethyl-1H-benz[e]indolium hydroxide (1 mol., 6.9 g.) and p-dimethylaminocinnamaldehyde (1 mol.+100%, 1 g.) were dissolved in acetic anhydride (20 ml.) and heated under reflux for five minutes. The reaction mixture was then chilled overnight and crystalline dye was filtered, washed on a Buchner funnel with acetone and dried. The yield of purified dye after two recrystallizations from methyl alcohol was 4.2 g. (44%), M.P. 220°-221° C.

Dye 2.—Anhydro-5-chloro-2-(4-p-dimethylaminophenyl-

1,3-butadienyl)-3,3-dimethyl-1-(4-sulfovutyl)-3H-indolium hydroxide

5



10

Anhydro-5-chloro-2,3,3-trimethyl-1-(4-sulfovutyl)-3H-indolium hydroxide (1 mol., 3.3 g.) and p-dimethylaminocinnamaldehyde (1 mol.+100% excess, 3.5 g.) were dissolved in acetic anhydride (25 ml.) and heated under reflux for twenty minutes. The reaction mixture was then chilled overnight and the crude dye thrown out of solution by the addition of an excess of ether with stirring. The ether was decanted from the sticky dye residue and the dye obtained in crystalline form by adding acetone with stirring. The crystalline dye was filtered, washed on the Buckner funnel with acetone and dried. After two recrystallizations from fifty percent methyl alcohol and water, the yield of purified dye was 1 g. (22%), M.P. 245°-246° C. dec.

Dye 3.—Anhydro-5-chloro-2-(4-p-methoxyphenyl-1,3-butadienyl)-3,3-dimethyl-1-(4-sulfovutyl)-3H-indolium hydroxide

Dye 3 was made like Dye 2 but by using the reactants anhydro-5-chloro-2,3,3-trimethyl-1-(4-sulfovutyl)-3H-indolium hydroxide (1 mol., 3.3 g.) and p-methoxycinnamaldehyde (1 mol.+100% excess, 3.0 g.), and reducing the concentration of acetic anhydride to 20 ml. The yield of purified dye was 1.3 g. (30%) M.P. 297°-298° C. dec.

Dye 4.—3-carboxymethylcarbamoyloxyethyl-2-(4-p-dimethylaminophenyl-1,3-butadienyl)-1,1-dimethyl-1H-benz[e]indolium iodide

40



45

1,1-dimethyl-2-(4-p-dimethylaminophenyl-1,3-butadienyl)-3-ethoxycarbonylmethylcarbamoyloxyethyl-1H-benz[e]indolium iodide (1 mol., 3.33 g.) and sodium hydroxide (1 mol.+100% excess, 0.4 g. in 2 ml. H<sub>2</sub>O) were dissolved in absolute ethyl alcohol (200 ml.) and the solution heated under reflux for ten minutes. The yellow precipitate that separated from the solution was then filtered, suspended in a small amount of water, the water suspension treated with acetic acid and the re-formed dye filtered off, washed with a small amount of acetone and dried. After two recrystallizations from 50% aqueous methyl alcohol the yield of pure dye was 2.0 g. (62%) M.P. 186°-187° dec.

Dye 5.—2-(4-p-dimethylaminophenyl-1,3-butadienyl)-3-ethoxycarbonylmethylcarbamoyloxyethyl-1,1-dimethyl-1H-benz[e]indolium iodide

1,1-dimethyl-2-(4-p-dimethylaminophenyl-1,3-butadienyl)-3-hydroxyethyl-1H-benz[e]indolium iodide (1 mol., 8 g.) and carbethoxymethylisocyanate (1 mol.+300% excess, 5 g.) were mixed in dry pyridine (75 ml.) and heated under reflux for one hour. The mixture was then chilled and the crystalline dye filtered off and dried. After two recrystallizations from methyl alcohol the yield of pure dye was 0.5 g. (50%) M.P. 230°-231° dec.

Dye 6.—2 - (4-p-dimethylaminophenyl-1,3-butadienyl)-3-hydroxyethyl-1,1-dimethyl-1H-benz[e]indolium iodide

3 - hydroxyethyl - 1,1,2-trimethyl-1H-benz[e]indolium bromide (1 mol., 18 g.) and p-dimethylaminocinnamaldehyde (1 mol. plus 10% excess., 10.3 g.) were mixed in absolute ethyl alcohol and the mixture heated under reflux for ten minutes. The mixture was then chilled and the dye precipitated as the iodide by adding sodium iodide with good stirring. The dye was then filtered off, stirred in a water suspension, filtered off, washed with a small amount of acetone and dried. After two recrystallizations from methyl alcohol the yield of pure dye was 12 g. (42%) M.P. 250°-250° dec.

Dye 7.—3 - carboxyethyl-2-(4-p-dimethylaminophenyl-1,3-butadienyl) - 1,1 - dimethyl-1H-benz[e]indolium iodide

3 - carboxyethyl - 1,1,2-trimethyl-1H-benz[e]indolium iodide (1 mol., 6.14 g.) and p-dimethylaminocinnamaldehyde were mixed in ethyl alcohol and the mixture heated under reflux for one hour. The mixture was then chilled and the crude dye filtered off, washed with a small amount of acetone and dried. After two recrystallizations from ethyl alcohol the yield of pure dye was 4.6 g. (54%), M.P. 174°-175° dec.

Dye 8.—Anhydro - 1,1-dimethyl-2-(4-p-dimethylaminophenyl - 1,3-butadienyl)-3-(3-sulfopropyl)-1H-benz[e]indolium hydroxide

Anhydro-3-(3-sulfopropyl)-1,1,2-trimethyl-1H-benz[e]indolium hydroxide (1 mol., 66.2 g.) and p-dimethylaminocinnamaldehyde (1 mol. plus 50% excess, 47.5 g.) were mixed in absolute ethanol (500 ml.) and heated under reflux for one hour. The mixture was then chilled over night and the crystalline dye filtered off, washed on a Buchner funnel with acetone and dried. The yield of purified dye after two recrystallizations from methanol was 51 g. (51%) M.P. 238°-239° C.

Dye 9.—Anhydro-2-(4-p-methoxyphenyl-1,3-butadienyl)-3,3-dimethyl-1-(4-sulfobutyl)-3H-indolium hydroxide

This dye was prepared by a method similar to that used for dye 2 but using the reactants anhydro-2,3,3-trimethyl-1-(4-sulfobutyl)-3H-indolium hydroxide (1 mol.) and p-methoxycinnamaldehyde (1 mol.+100% excess), and reducing the concentration of acetic anhydride to 20 ml.

Dye 10.—Anhydro-2-(4-p-dimethylaminophenyl-1,3-butadienyl)-3,3-dimethyl-1-(4-sulfobutyl)-3H-indolium hydroxide

This dye was prepared by a method similar to that used to make dye 2 but using as the reactants anhydro-2,3,3-trimethyl - 1-(4-sulfobutyl)-3H-indolium hydroxide (1 mol.) and p-dimethylaminocinnamaldehyde (1 mol.+100% excess).

Dye 11.—Anhydro-2-(4-p-dimethylaminophenyl-1,3-butadienyl)-1,1-dimethyl-3-(3-sulfobutyl)-1H-benz[e]indolium hydroxide, monosulfonated



1,1,2-trimethyl-1H-benz[e]indole - monosulfonated (1 mol., 5.78 g.) and 2,4-butanedisulfone (sufficient excess to form a mobile mixture) were mixed and heated over a free

75

free flame until the viscous mixture turned brownish-black in color. The mixture was then cooled and the anhydro-3 - (3 - sulfobutyl)-1,1,2-1H-benz[e]indolium hydroxide-monosulfonated precipitated as a grey solid by treating with an excess of acetone and stirring. At this point the hydroscopic grey solid was filtered off, dissolved in refluxing ethyl alcohol (100 ml.), p-dimethylaminocinnamaldehyde (1 mol., 3.5 g.) added and the mixture heated under reflux for fifteen minutes. The mixture was then chilled and the crude dye precipitated from solution by turning the mixture into acetone (300 ml.) with stirring. The solid dye was filtered off, washed with acetone and dried. After two recrystallizations from aqueous methyl alcohol and acetone the yield of pure dye was 3.5 g. (31%); melting point 289°-290° C. dec.

Dye 12.—Anhydro-3-carboxyethyl-2-(4-p-dimethylaminophenyl - 1,3-butadienyl)-1,1-dimethyl-1H-benz[e]indolium hydroxide, monosulfonated; pyridine salt



1,1,2-trimethyl-1H-benz[e]indole - monosulfonated (1 mol., 5.78 g.) and propiolactone (sufficient excess to form a mobile mixture) were mixed and heated over a free flame until the solid went into solution and the solution turned amber in color. The mixture was then removed from heat and reaction took place causing the solution to turn dark in color with a vigorous evolution of heat. The dark viscous mass was cooled, stirred with an excess of ether, ether decanted and the sticky residue dissolved in refluxing ethyl alcohol (200 ml.). At this point p-dimethylaminocinnamaldehyde (1 mol., 3.5 g.) was added and the mixture heated under reflux for ten minutes. The solid dye was collected and after two recrystallizations from ethanol/pyridine the yield of pure dye was 45 g. (43%), M.P. 226°-227° C. dec.

Dye 13.—2-[4-p-dimethylaminophenyl-1,3-butadienyl]-1-ethyl-3,3-dimethyl-3H-indolium iodide

This dye was prepared by a reaction similar to that used to prepare Dye 6 excepting that 1,1,2-trimethyl-indolenine ethiodide and p-dimethylaminocinnamaldehyde were used. The yield of purified dye was 32%, M.P. 238°-239° C. with dec.

The preparation of typical intermediates used in making our dyes will further illustrate our invention.

3-hydroxyethyl-1,1-dimethyl-1H-benz[e]indolium bromide

1,1,2 - trimethyl - 1H - benz[e]indole (1 mol., 10.4 g.) and 2-bromoethanol (1 mol., 6.25 g.) were mixed and heated on a steam bath for twenty-four hours. The hard cake that formed was ground under ether, suspended in acetone, filtered and dried. The yield was 15 g. (90%), M.P.=159°-160° dec.

65 The corresponding iodide salt was prepared from the bromide by double decomposition with sodium iodide.

3-carboxyethyl-1,1,2-trimethyl-1H-benz[e]indolium iodide

70 1,1,2-trimethyl-1H-benz[e]indole (1 mol. plus 100% excess., 20.9 g.) and  $\beta$ -iodopropionic acid (1 mol., 10 g.) were mixed and heated on a steam bath for 12 hours. The product was then washed with ether, refluxed in acetone, filtered and dried. The yield of light tan solid was 14 g. (70%) M.P. 181°-182° dec.

Anhydro-3-(4-sulfonylbutyl)-1,1,2-trimethyl-1H-benz[e]indolium hydroxide, and anhydro-3-(3-sulfonylpropyl)-1,1,2-trimethyl-1H-benz[e]indolium hydroxide were prepared by the methods described in Heseltine and Brooker, U.S. Patent 2,895,955, issued July 21, 1959. Anhydro-2,3,3-trimethyl-1-(4-sulfonylbutyl)-3H-indolium hydroxide was prepared from 1,1,2-trimethylindole by reaction described in U.S. Patent 2,895,955. The corresponding 5-chloro derivative was prepared in the same manner but starting with 5-chloro-2,3,3-trimethyl-3H-indole.

Our dyes have light-absorbing characteristics that make them valuable for use in filter and antihalation layers of photographic elements. These characteristics are illustrated in Table I below.

TABLE I

| Dye Number: | Maximum light absorption by dye occurs at a wavelength in $\mu$ of |
|-------------|--------------------------------------------------------------------|
| 1           | 615                                                                |
| 2           | 630                                                                |
| 3           | 470                                                                |
| 4           | 625                                                                |
| 5           | 625                                                                |
| 6           | 605                                                                |
| 7           | 620                                                                |
| 13          | 610                                                                |

Our butadienyl dyes are distinguished from other butadienyl dyes by having maximum light absorption at wavelengths that are considerably longer than other butadienyl dyes that are outside our invention. Furthermore, the increase in depth of color with the introduction of a vinylene group is much larger with our indolenine and benz[e]indole dyes than it is with other typical nuclei used in styryl dyes. The following table illustrates.

TABLE II.—ADSORPTION MAXIMA OF P-DIMETHYLAMINOSTYRYL AND P-DIMETHYLAMINOBUTENYLIDENE DYES

| Heterocyclic Nucleus                                                                | Styryl Dye<br>( $\mu$ ) | Butadienyl<br>Dye ( $\mu$ ) | Increase in Depth<br>of Color With<br>Introduction of<br>One Vinylene<br>Group ( $\mu$ ) |
|-------------------------------------------------------------------------------------|-------------------------|-----------------------------|------------------------------------------------------------------------------------------|
|  | 532.5                   | 564.0                       | 31.5                                                                                     |
|  | 525.0                   | 556.0                       | 31.0                                                                                     |
|  | 560.0                   | 615.0                       | 55.0                                                                                     |
|  | 557.0                   | 633.0                       | 76.0                                                                                     |

These data show that of the higher vinylogs only the immediate dyes absorb at wavelengths longer than 600  $\mu$ . It is unexpected that the immediate dyes would have shifts in the spectral absorption as high as 70  $\mu$  from the corresponding styryl (lower vinylog) dye when the shift in spectral absorption of butadienyl dyes outside our invention and their lower vinylogs is only about 31  $\mu$ .

Our dyes are readily soluble in water because of their ionic nature and are thus readily incorporated in hydrophilic colloids such as gelatin, polyvinyl alcohols, albumen, and casein which are usually used for filter and antihalation layers of photographic materials. A stock solution may be made of the dye to be used and this 15 can be added to the hydrophilic colloid solution before it is coated.

The concentration of dye in the hydrophilic colloid may be varied considerably depending upon the product 20 in which the filter or antihalation layer is to be used. The proper amount of dye to be used for a given product can be determined by methods well known in the art.

In the accompanying drawing, FIGURES 1 and 2 are 25 enlarged sectional views of photographic elements having filter layers or antihalation layers made according to our invention. As shown in FIGURE 1, a support 10 of any suitable material such as cellulose acetate, cellulose nitrate, synthetic resin materials or opaque materials such as paper, is coated with an emulsion layer 11 and an over-coating layer 12 comprising a hydrophilic colloid such as gelatin and a butadienyl dye of our invention.

FIGURE 2 illustrates a multilayer photographic element 30 for color photography in which the support 10 is coated with sensitive layers 13, 14 and 15 which record light of the red, green and blue regions of the spectrum respectively. Between the emulsion layers 14 and 15 there is a filter layer 16 containing gelatin and a yellow butadienyl dye. This filter layer serves a purpose well known in color photography of preventing exposure of a lower layer of the element by light which the filter layer absorbs. The dye may also absorb light in other regions such as the ultraviolet region on the spectrum.

FIGURE 3 represents a film having an antihalation 35 layer containing a dye of our invention. As shown therein, the support 10 carries an emulsion layer 11 on one side and an antihalation layer 17 containing a butadienyl dye on the opposite side.

FIGURE 4 represents a film having under the emulsion 40 an antihalation layer containing a dye of our invention. As shown, the support 10 carries an antihalation layer 18 which has been overcoated with emulsion layer 11. This antihalation layer serves the well-known purpose of absorbing light passing through the layer and its reflection from the surface of the support back to the emulsion layer.

These dyes can be advantageously used in the preparation 45 of photographic light screening layers by dissolving the dyes in water, or a mixture of alcohol and water, and adding the resulting solution to an aqueous hydrophilic colloidal solution, or to a hydrophobic colloidal solution, e.g., cellulose acetate phthalate or the cellulose ester of dimethylaminoacetic acid before coating.

Examples of the use of the dyes of our inventions are 50 illustrated as follows:

One mg. of Dye 1 was dissolved in 5 ml. of methanol 55 and diluted to 20 ml. with water. This solution was added to 10 ml. of a 10 percent photographic gelatin solution containing 0.5 ml. of 15% saponin solution. The mixture was coated on a suitable support at a thickness that contained from ten to twenty mg. of dye per square foot.

A layer of alkali-removable cellulose acetate phthalate 60 coated over cellulose triacetate sheeting was followed by an overcoat of the following composition: 1.0% of Dye 2 in a mixture of 95% alcohol and 5% water.

A layer of alkali-removable cellulose acetate phthalate 65 was coated over cellulose triacetate followed by a dye

coat of the following composition: 0.4% anhydro-5-chloro - 2-p-dimethylaminostyryl - 3,3 - dimethyl-1-(4-sulfobutyl)-3H-indolium hydroxide, 1.0% of Dye 2 from alcohol-water.

The following examples will illustrate more fully how our dyes may be used in preparing light absorbing filter layers.

#### Example 1

1.5 grams of Dye 1 were dissolved in 37.5 ml. of water and this solution was added to 4.5 liters of 5% aqueous gelatin. This mixture was then coated as an antihalation backing on the reverse side of a support which has been coated with a photographic silver halide emulsion layer.

After exposure of the photographic element in the usual manner, development of the exposed material in a developer having the following composition:

|                                |            |      |
|--------------------------------|------------|------|
| N-methyl-p-aminophenol sulfate | -----grams | 2    |
| Sodium sulfite (desiccated)    | -----do    | 90   |
| Hydroquinone                   | -----do    | 8    |
| Sodium carbonate monohydrate   | -----do    | 52.2 |
| Potassium bromide              | -----do    | 5    |
| Water to make                  | -----liter | 1    |

followed by fixation in a conventional sodium thiosulfate fixing bath resulted in complete removal of the dye from the photographic element.

#### Example 2

A photographic element made as in Example 1, but using Dye 4 in place of Dye 1 was exposed. No dye color was evident in this element after development, and fixing with the solutions used in Example 1.

#### Example 3

A mixture of Dye 1 and aqueous gelatin solution as prepared in Example 1 was coated over a light sensitive silver halide emulsion layer on a conventional support.

After exposure of the photographic element in the usual manner, development and fixing of the exposed material in the solutions of Example 1 resulted in a complete removal of the dye color from the light filtering layer over the developed image.

#### Example 4

Similarly, the other dyes of our invention can be used in light filtering layers as in Example 3.

The above examples show the use of our dyes in anti-halation layers and in layers overcoating the light sensitive silver halide emulsion layer; they can also be coated between light sensitive silver halide layers in multilayer photographic elements.

The novel dyes of our invention are characterized by being readily water soluble and readily bleachable by ordinary photographic developers and processing solutions. These properties make our dyes valuable for use in making light sensitive photographic elements. Our dyes are particularly valuable in light absorbing filter layers either coated over the silver halide emulsion layers, or coated between light sensitive silver halide layers, or coated on either side of the support on which the light sensitive silver halide emulsion layers are coated.

The invention has been described in detail with particular reference to preferred embodiments thereof, but it will be understood that variations and modifications can be effected within the spirit and scope of the invention as described hereinabove and as defined in the appended claims.

We claim:

1. A photographic element comprising a support having coated thereon at least one light-sensitive silver halide

emulsion layer, said element having a light-absorbing layer containing a dye having the formula:



wherein L represents a group selected from the class consisting of the hydrogen atom, and a halogen atom; Y and Y<sub>2</sub> each represent a member selected from the class consisting of a hydrogen atom, the non-metallic atoms which when taken together form a fused ring attached to the indolenine ring; R and R<sub>1</sub> each represent a member selected from the class consisting of the hydrogen atom, an alkyl group, and R and R<sub>1</sub> together represent the non-metallic atoms necessary to complete a cycloalkane group; R<sub>2</sub> represents an alkyl group; X<sup>⊖</sup> represents an acid anion; n represents an integer of from 1 to 2 such that n represents the integer 1 only when R<sub>2</sub> contains a group selected from the class consisting of the carboxy group, and the sulfo group; and Z represents a member selected from the class consisting of an aminoaryl group, an alkoxyaryl group and a hydroxyaryl group.

2. A photographic element of claim 1 in which the said light-absorbing layer is coated over the said light-sensitive layer.

3. A photographic element of claim 1 in which the said light-absorbing layer is coated between the said support and the said light-sensitive layer.

4. A photographic element of claim 1 in which the said light-absorbing layer is coated on one side of the said support and the said light-sensitive layer is coated on the other side of the said support.

5. A photographic element of claim 1 in which the said light-absorbing layer is coated between two light-sensitive layers.

6. A photographic element of claim 1 containing anhydro - 2 - (4 - p - dimethylaminophenyl - 1,1 - dimethyl-1,3 - butadienyl) - 3 - (4 - sulfobutyl) - 1H - benz[e]indolium hydroxide.

7. A photographic element of claim 1 containing 3-carboxyethyl - 2 - (4 - p - dimethylaminophenyl - 1,3-butadienyl) - 1,1 - dimethyl - 1H - benz[e]indolium iodide.

8. A photographic element of claim 1 containing anhydro - 5 - chloro - 2 - (4 - p - dimethylaminophenyl - 1,3-butadienyl) - 3,3 - dimethyl - 1 - (4 - sulfobutyl) - 3H-indolium hydroxide.

9. A photographic element of claim 1 containing anhydro - 3 - carboxyethyl - 2 - (4 - p - dimethylaminophenyl - 1,3 - butadienyl) - 1,1 - dimethyl - 1H - benz[e]indolium hydroxide; monosulfonated pyridine salt.

10. A photographic element of claim 1 containing 3-carboxymethylcarbamoyloxyethyl - 2 - (4 - p - dimethylaminophenyl - 1,3 - butadienyl) - 1,1 - dimethyl - 1H - benz[e]indolium iodide.

#### References Cited

##### UNITED STATES PATENTS

3,095,303 6/1963 Sprague et al. ----- 96-33  
3,102,810 9/1963 Sprague et al. ----- 96-33

##### OTHER REFERENCES

P. Ruggli, and P. Jensen, *Helv. Chim. Acta* 18, pp. 632, 633, 1935.

70 NORMIN G. TORCHIN, *Primary Examiner*.

R. H. SMITH, *Assistant Examiner*.